

Aug. 10, 1926.

1,595,436

H. M. WALL

ROPE STRUCTURE

Filed July 2, 1923

*Fig. 1.*



*Fig. 2.*



INVENTOR

Harold M. Wall

BY

Frank J. Hart

ATTORNEY

Patented Aug. 10, 1926.

1,595,436

# UNITED STATES PATENT OFFICE.

HAROLD M. WALL, OF BEVERLY, NEW JERSEY, ASSIGNOR TO WALL ROPE WORKS, INC.,  
OF NEW YORK, N. Y., A CORPORATION OF NEW JERSEY.

## ROPE STRUCTURE.

Application filed July 2, 1923. Serial No. 648,931.

This invention relates generally to rope or cordage construction, and more particularly to the structure of the individual strands which are twisted together to form the completed product.

The invention includes a strand formation of the general type in which bodies or masses of fibres form strand core members which are wound or wrapped with covering yarn.

In strands of this general construction which have been heretofore manufactured, the strand cores have consisted of a single body of untwisted fibres or of general groups; e. g., two or more groups twisted in the same direction and these groups then twisted and laid together; or of a multiplicity of twisted interior yarns. The first mentioned structure is lacking in firmness and compactness, while the second and third are characterized by excessive detrimental internal friction.

In the present invention I have succeeded in eliminating the various objectionable features referred to by making use of a strand core consisting of two or more bodies of fibre between which there is relatively negligible frictional contact. The reduction in friction is achieved in great part by the particular relation between the core parts which differ from the prior construction in that they are not twisted in the same direction. I have found that advantageous results can be achieved by twisting the core parts in opposite directions. In the construction referred to it will be seen that a balanced construction is obtained in which there is no tendency for the rope to kink or twist on itself. The reduced number of parts reduces the shearing action that is present where a multiplicity of yarns is used, and the tensile strength of the strand and rope is increased.

The construction provides also for a less number of twists or turns per unit length, and thereby increases the pliability of the construction. In addition, the characteristic twist and relation of the core parts provide a method of identification of the product.

In the drawings, in which a preferred form of the invention has been selected for illustration,

Figure 1 is a view of a section of rope embodying the invention and opened out at one end to show the internal construction; and

Figure 2 is a sectional view of the rope shown in Figure 1 taken on the line 2—2. 55

Referring to the drawings for a more detailed description of the invention, a section of rope embodying the invention is shown at 10, and is made up of three strands 11 twisted together to form the final product. 60 While a three strand rope is shown for the purpose of illustration, it will be clear that a lesser or greater number of strands may be utilized without departure from the invention. 65

The distinguishing feature of the invention resides in the construction of the individual strands 11 which are used to form the rope or cable 10. The strands are of the cored type, that is, they are made up of 70 bodies or bundles 12 of fibres enclosed by a covering of yarn 13.

The core parts 12 consist of relatively large bundles or groups of fibres having, in the instance illustrated, a twist in opposite directions, that is, the fibres of one of the core parts are twisted in a right-hand or clockwise direction and those of the other core part in a left-hand or counter-clockwise direction, from the standpoint of an observer 80 looking along the length of the strands.

I have found that by combining two or more bodies of fibres, the fibres of one body being twisted in an opposite direction from the direction of twist in another body, a 85 construction is provided in which the several parts balance each other and do away with the tendency to unwind or untwist. The result of this is that the strand and consequently the rope including the structure of 90 strand referred to, is free from the tendency to kink or to spin when a length of rope so constructed is used to suspend a body. By reason of the twist which is characteristic of the individual core parts 12, the ultimate 95 rope or cable possesses a high degree of pliability, and at the same time the core parts provide a compact body having minimum frictional contact between the members and possessing a relatively high degree of tensile strength. In addition the peculiar relation that exists between the core parts obviates the tendency to shear that might otherwise exist. 100

The strand 11 is completed by wrapping 105 the core parts 12 with the covering yarns 13,

already referred to; and a rope or cable may be formed by twisting together two or more of such strands in a known manner.

I claim:

- 5 1. A rope construction made up of a plurality of strands twisted together, each strand including a plurality of distinct groups of fibers, each group of fibers being twisted in a different direction from the fibers in the adjacent group, and a yarn covering wound into place on each of said strands.
- 10 2. A rope construction made up of a plurality of strands twisted together, each strand including a plurality of distinct groups of fibers, each group of fibers being twisted in a different direction from the fibers in the adjacent group, said groups of fibers being twisted together, and a yarn covering on each strand.
- 15 3. A rope construction made up of a plurality of strands twisted together, each strand having a core composed of a plurality of distinct groups of fibers, all of the fibers in one group being twisted in the opposite direction to the twist of the fibers in the adjacent group, said groups of fibers being twisted together to form the core, and a yarn covering on each strand.
- 20 4. A rope construction made up of a plurality of strands twisted together, each strand including a plurality of distinct bodies of fibers, said bodies being twisted in opposite directions and further intertwined to

form the core of the strand, and a yarn covering on each strand.

5. A rope structure comprising a plurality of intertwined strands, each strand consisting of distinct bodies of fibers respectively twisted in opposite directions, and a yarn covering wound into place on each strand.

6. A rope structure comprising a plurality of intertwined strands, each strand consisting of distinct bodies of fibers respectively twisted in opposite directions, and a yarn covering wound into place on each strand, said bodies of fibers being twisted together.

7. A rope structure comprising a plurality of strands twisted together, each strand consisting of two or more relatively large and distinct bundles of fibers, the fibers in one bundle being twisted in one direction and the fibers in the adjacent bundle being twisted in the opposite direction, the several bundles being twisted together to form the core of the strand, and a plurality of yarns wound in covering relation on each of the strands.

8. A rope strand comprising a plurality of distinct bodies of fibers intertwined to form a core for the strand, all of the fibers in one body being twisted together and in the opposite direction to the twist of the fibers in the adjacent body, and a yarn covering on each strand.

In testimony whereof I affix my signature,

HAROLD M. WALL.